

## UNITED STATES PATENT OFFICE

2,577,298

## FLASHLESS POWDER SHEET

Alpheus M. Ball, Wilmington, Del., assignor, by  
mesne assignments, to the United States of  
America as represented by the Secretary of War

No Drawing. Application May 3, 1946,  
Serial No. 667,128

7 Claims. (Cl. 102—98)

**1**  
This invention relates to smokeless powder and, more particularly, to a solventless-type smokeless powder sheet suitable for use in trench mortars.

Smokeless powders, suitable for use as propellents in trench mortars and particularly the 4.2-inch chemical mortar, are required to give a certain specified muzzle velocity to the mortar projectile while at the same time maintaining the pressure within the barrel within certain specified limits. In the case of the 4.2-inch chemical mortar, the velocity required is in the neighborhood of 820 feet per second plus or minus 10 feet per second and the maximum pressure in the neighborhood of 12,500 pounds per square inch.

Considerations influencing these requirements are the length and thickness of the mortar barrel and the space available for the propellant. It will be appreciated, in view of the limited space available for the powder charge, that the composition and thickness of the powder sheets must be closely regulated to produce the required muzzle velocity within the confining limits of the length of the barrel while at the same time maintaining the pressure below a point which would tend to rupture or distort the walls of the barrel.

Another requirement for powders of this type is that they be of a nature such that they lend themselves to manufacture into sheets by a rolling operation as customarily practiced in the production of mortar-type powders. Although not a requirement, it is also highly desirable and somewhat essential that such powders be substantially flashless when fired. The shortness of the mortar barrel together with the ballistic requirements make this very difficult of attainment.

At the present time these requirements are met in part by a mortar-type powder sheet having a thickness in the neighborhood of 0.025 inch, a calorific value of about 1250 calories per gram, and a composition comprising nitrocellulose and nitroglycerin in combination with other suitable and desirable materials. A characteristic composition of this type is nitrocellulose about 52%, nitroglycerin about 43%, diphenylamine about 0.60%, diethyl phthalate about 3%, and potassium nitrate about 1.25%. Although such powder sheets give the desired ballistic properties, they are subject to the disadvantage that when fired from a mortar and particularly the 4.2-inch chemical mortar they produce a flash which may be seen at night from a long distance. Such a flash is readily picked up by an alert enemy and usually results in enemy fire which may be effective

enough to destroy one or more mortars and kill or wound the operating personnel.

Previous attempts to eliminate the muzzle flash of mortar-type powders, as by varying the composition of the powder, adding flash depressants, etc., have been generally unsatisfactory. The utilization of powders having lower calorific values has not been considered feasible, since skilled workers in the art have supposed that a powder of high calorific value was necessary in order to obtain required muzzle velocities within fixed pressure limits. Furthermore, known powder compositions of lower calorific value are not suitable for use as mortar-type powders, since their nature is such that they are not susceptible of manufacture in accordance with the requirements of such powder; i. e., rolling into sheets, and additionally do not give the necessary ballistic properties such as, for example, the requisite muzzle velocity. It would be expected that the requisite muzzle velocity could, of course, be obtained by a relatively large increase in the weight of the powder charge. However, when this is attempted excessive pressures are likely to be encountered and it frequently becomes necessary, in view of the limited propellant charge space available in most mortars, to redesign the mortar to accommodate the increased charge. This always results in a lowering of production which is particularly critical in time of war.

**2**  
The above disadvantages are overcome by this invention by providing a mortar-type smokeless powder sheet having a thickness substantially less than that hitherto used, a calorific value of from 900-1100 calories per gram, which produces substantially no flash when fired in a 4.2-inch chemical mortar, and which fulfills all ballistic requirements of this type of powder without requiring any modification of existing mortar construction.

In accordance with the present invention the mortar-type smokeless powder sheets may comprise from about 50% to about 58% nitrocellulose (12.2% to 13.4% nitrogen content), about 12% to about 44% nitroglycerin, about 2% to about 10% of a cooling plasticizer, from about 0% to about 35% of diethanol nitramine dinitrate, a small amount of stabilizer such as diphenylamine or ethyl centralite, a small amount of inorganic salt to facilitate ignition and regulate burning, and in some cases a small amount of a desensitizer. The proportion of the cooling plasticizer is coordinated with the proportions of the other materials to produce a powder having a calorific value between 900 and 1100 calories per gram. Suitable formulations are given hereinafter in

Examples I and II. The powder sheets may be manufactured in accordance with a process which will generally include the steps of mixing, drying, rolling into sheets, and sewing, slitting, and punching the sheets into packs, bundles, etc., as required.

The thickness of the finished powder sheets will vary with the size of the mortar and will be coordinated with the diameter of the bore and the length of the barrel so that the requisite ballistics are obtained without a substantial increase in the weight of the charge over that necessary in powders of higher calorific value now used for this purpose. Where quick burning is required, as in the case of a mortar with a relatively short barrel, the sheets should be relatively thin. Where longer burning is suitable, as in the case of a comparatively long barrel, the sheets may be thicker. Thus, for the 4.2-inch chemical mortar, the thickness of the sheets may vary from about 0.012 inch to about 0.020 inch but is preferably about 0.016 inch. For the 60 mm. trench mortar the sheet thickness may be as little as 0.003 inch.

In all cases the thickness of the sheets will be substantially less than and of the order of about one-half the thickness of those utilized heretofore for this purpose. This is made possible by the low calorific value of the improved powder composition of this invention.

The following is an example of a preferred powder made according to this invention.

*Example I*

| Material:                 | Percentage<br>by weight |
|---------------------------|-------------------------|
| Nitrocellulose (13.25% N) | 55.00                   |
| Nitroglycerin             | 33.65                   |
| Diphenylamine             | 0.60                    |
| Diethyl phthalate         | 9.50                    |
| Potassium nitrate         | 1.25                    |
| Methyl cellulose (added)  | 0.20                    |

The ingredients were mixed, dried, rolled into sheets 0.016 inch thick, and the sheets cut, sewed, slit, and punched into packs, bundles, and half bundles for the 4.2-inch chemical mortar. This powder had a calorific value of 1007 calories per gram, and produced substantially no flash when fired at night in the 4.2-inch mortar. A charge weight of 3284 grains of this powder, when utilized to fire a projectile from a 4.2-inch mortar, produced a mean muzzle velocity of 812 feet per second and a mean pressure of 10,300 pounds per square inch. 2958 grains of a standard powder having a calorific value of 1250 calories per gram produced a mean muzzle velocity of 817 feet per second and a mean pressure of 11,600 pounds per square inch under similar conditions.

Another preferred embodiment of this invention is given by the following example.

*Example II*

| Material:                     | Percentage<br>by weight |
|-------------------------------|-------------------------|
| Nitrocellulose (12.60% N)     | 51.00                   |
| Nitroglycerin                 | 15.00                   |
| Ethyl centralite              | 1.50                    |
| Diethyl phthalate             | 3.25                    |
| Potassium nitrate             | 1.25                    |
| Diethanol nitramine dinitrate | 28.00                   |

This powder was mixed by the slurry method rather than the standard Schrader method. The nitrocellulose was suspended in ten times its weight of water heated to 85° C. and the nitroglycerin added while stirring. The centralite and

diethyl phthalate were added and the whole stirred for 15 minutes. The diethanol nitramine dinitrate was added, while stirring, and the mixture cooled to 57° C. and held there for fifteen minutes. Then the whole was cooled to below 45° C. and filtered. The material was then dried, and rolled into sheets 0.016 inch thick in accordance with the usual procedure for manufacturing trench mortar powder.

This powder had a calorific value of 1036 calories per gram and produced substantially no flash when fired at night in the 4.2-inch mortar. A charge of 3200 grains produced a mean muzzle velocity of 807 feet per second and a mean pressure of 9925 pounds per square inch when fired in the 4.2-inch mortar. This compares favorably with a mean velocity of 817 feet per second and a mean pressure of 9200 pounds per square inch obtained with 2956 grains of a standard powder under similar circumstances.

From the above examples it will be seen that there has been provided a mortar-type powder of low calorific value which is substantially flashless when fired in a mortar at night, and which meets all ballistic requirements of a powder of this type.

In practicing this invention the nitrocellulose content of the powder should be held within the range of from about 50% to about 58%. Utilization of percentages above and below this range is not satisfactory, since the resultant powder is not suitable for rolling into sheets as required in the manufacture of mortar-type powder. The nitrogen content of the nitrocellulose used may vary from about 12.2% to about 13.4% but is preferably within the range from about 12.6% to about 13.3%.

The nitroglycerin and cooling plasticizer are incorporated in proportions to obtain a calorific value of 900 to 1100 calories per gram with the amount of nitrocellulose used. Thus, when the percentage of nitrocellulose is increased with respect to the percentage of nitroglycerin, the percentage of cooling plasticizer may be decreased. The nitroglycerin will be present in amounts ranging from about 12% to about 44% and the cooling plasticizer in amounts ranging from about 2% to about 10%. The preferred cooling plasticizer is diethyl phthalate. Other suitable cooling plasticizers, such as dimethyl phthalate, dibutyl phthalate, triacetin, trinitrotoluene, dinitrotoluene, and a partial substitution of any of these with ethyl centralite may be used alone or in suitable combinations to produce the desired low calorific value.

From about 0% to about 35% of diethanol nitramine dinitrate may desirably be incorporated in the mixture to replace a portion of the nitroglycerin. In such cases the percentage of nitroglycerin may be reduced to but not below about 12% and the cooling plasticizer to about 2% to give the desired calorific value.

As a stabilizing agent it is desirable to use either diphenylamine or ethyl centralite. The diphenylamine should be present in amounts from about 0.5% to about 1% and preferably about 0.60%. From about 0.5% to about 1.50% of the ethyl centralite is normally adequate to insure satisfactory storage life of the powder, but an additional amount may be used on account of its plasticizing properties and also on account of its cooling effect as indicated by its negative partial calorific value. Thus, when incorporated for these additional purposes, a total of up to about 8% may be used with a consequent

reduction in the amount of cooling plasticizer required. In most cases, however, it is preferable not to use more than about 5%.

Other stabilizers which may be used are carbazole, beta-nerolin, or similar compounds capable of reacting with oxides of nitrogen.

It is preferred to incorporate in the powder minor amounts of a potassium salt such as, for example, from about 0.75% to about 1.50% and preferably about 1.25% of potassium nitrate. This salt facilitates ignition of the powder and helps to regulate burning. Although potassium nitrate is a preferred salt for this purpose, other salts, and preferably potassium salts, such as potassium sulfate, are satisfactory. Salts of bi- and poly-valent cations are also satisfactory. In general, salts of the univalent type are the least satisfactory since they appear to adversely effect the stability of the powders at elevated temperatures, while salts of other valence types are inactive in so far as any effect on the stability of the powders is concerned and, therefore, are preferred from these considerations.

In some cases, as in the mixture of Example I, it is desirable to add a very minor amount in the order of about 0.20% of a desensitizing material such as methyl cellulose.

The smokeless powder of this invention is useful as a propellant in trench mortars and particularly the 4.2-inch chemical mortar. By virtue of its lower calorific value of 900-1100 calories per gram and its reduced sheet thickness properly coordinated with the bore and length of the mortar barrel, it is possible to obtain a flashless discharge without substantial increase in charge weight while at the same time meeting all ballistic requirements. The advantages of this invention may, therefore, be realized without modification of the structure of the mortar.

Where in the specification and appended claims the term "calorific value" is used, it is meant the heat of explosion in calories per gram obtained when a sample of the substance is burned in a bomb calorimeter, for example, of the Parr oxygen bomb type, in an inert atmosphere so as to duplicate as closely as possible the state of oxidation prevailing in the weapon.

What I claim and desire to protect by Letters Patent is:

1. A flashless mortar-type smokeless powder sheet having a thickness of between about 0.003 inch and about 0.020 inch and comprising nitrocellulose in an amount from about 50% to about 58%, nitroglycerine from about 12% to about 44% and from about 2% to about 10% of a cooling plasticizer having a negative calorific value chosen from the group consisting of diethyl phthalate, dimethyl phthalate, dibutyl phthalate, triacetin, trinitrotoluene and mixtures thereof, the nitroglycerine and cooling plasticizer being in such proportions that the powder sheet has a calorific value between about 900 to 1100 calories per gram.

2. The flashless powder sheet of claim 1 containing in addition diethanol nitramine dinitrate in an amount up to 35% of the total weight of said sheet.

5 3. The powder sheet of claim 1 containing in addition as an auxiliary cooling plasticizer ethyl centralite, the total amount of said cooling plasticizer not exceeding 10%.

10 4. The flashless mortar-type smokeless powder sheet of claim 1 containing in addition between about 0.05% and 1.5% of a stabilizing agent.

5 5. The powder sheet of claim 4 in which the stabilizing agent is chosen from the group consisting of diphenylamine, ethyl centralite, carbazole, and beta-nerolin.

15 6. A flashless mortar-type smokeless powder sheet having a thickness between about 0.003 inch and about 0.020 inch and comprising by weight about 55% nitrocellulose (13.25% N), about 33.65% nitroglycerin, about 9.50% diethyl phthalate, and a stabilizer, the ingredients being proportioned to give a powder sheet having a calorific value between about 900 and 1100 calories per gram.

20 7. A flashless mortar-type smokeless powder sheet having a thickness between about 0.003 inch and about 0.020 inch and comprising by weight about 51% nitrocellulose (12.60% N), about 15% nitroglycerin, about 3.25% diethyl phthalate, about 28% diethanol nitramine dinitrate and a stabilizer, the ingredients being proportioned to give a powder sheet having a calorific value between about 900 and 1100 calories per gram.

ALPHEUS M. BALL.

#### REFERENCES CITED

The following references are of record in the file of this patent:

#### UNITED STATES PATENTS

| Number       | Name       | Date          |
|--------------|------------|---------------|
| 1,757,584    | Olin       | May 6, 1930   |
| 1,788,438    | Norton     | Jan. 13, 1931 |
| 45 1,838,345 | Woodbridge | Dec. 29, 1931 |
| 2,003,914    | Whitworth  | June 4, 1935  |
| 2,008,889    | Wagner     | July 23, 1935 |
| 2,120,324    | Dickerman  | June 14, 1938 |
| 2,440,267    | Hale       | Apr. 27, 1948 |
| 50 2,440,327 | Crawford   | Apr. 27, 1948 |

#### FOREIGN PATENTS

| Number     | Country       | Date          |
|------------|---------------|---------------|
| 122,509    | Great Britain | Jan. 30, 1919 |
| 55 621,685 | Great Britain | Apr. 14, 1949 |

#### OTHER REFERENCES

- Meyer, "Science of Explosive," (1943), pages 26 and 104, Crowell Publishing Company, New York. (Copy in Scientific Library.)
- 60 "Elements of Ammunition" by Maj. Theodore C. Ochart, copyright 1946 by John Wiley and Sons, New York, New York. Published March 21, 1946. (Copy in Division 70.) Page 27.